

## UNITED STATES PATENT OFFICE

2,554,089

## STRUCTURAL COVERING MATERIAL

Michele Croce, Evanston, Ill., assignor to Certain-Teed Products Corporation, Chicago, Ill., a corporation of Maryland

No Drawing. Continuation of abandoned application Serial No. 387,065, April 5, 1941. This application June 28, 1946, Serial No. 680,086

2 Claims. (Cl. 117—140)

1

This invention relates to covering materials, especially coverings which are intended to be exposed to the weather. The invention particularly relates to exterior coverings for walls and roofs which, in addition to affording weather protection, have structural characteristics in themselves.

This application is being filed as a continuation of my copending application, Serial No. 387,065, filed April 5, 1941, and now abandoned.

Covering materials, such as sheet roofing, made with a felt base impregnated with a weather resisting material such as asphalt, and in most cases coated with a weather resisting coating and surfaced with a comminuted surfacing material have been used in many forms. For the impregnating materials, commonly referred to in the roofing art as "saturants," bituminous materials or asphalts having particular properties have been selected in order that the impregnated sheet shall not be unduly subject to changes in temperature occurring with the seasons which would cause the saturant to bleed out of the sheet and thus damage or mar the roofing or the supporting structure. Similar care in selection is used in connection with the water resisting coating applied on such "saturated" felt base sheets to prevent sliding or other changes in the coating with temperature which would produce defects in the product.

This desirable quality of such saturants or coating materials, particularly asphalts, is known as low thermal susceptibility. It is, however, not possible with asphalts and bituminous materials ordinarily available, to secure a condition of susceptibility approaching the ideal, or even approximating that which is desirable. The result is that in most cases a compromise is adopted by virtue of which there is used a bituminous material or asphalt which under low temperatures, say below 50° F., is hard though somewhat brittle but at high temperatures, say above 100° F., is somewhat softened although not to the degree that it will readily flow. With bituminous materials, particularly asphalt, the range of temperatures within which such qualities may be secured is generally between 40° and 150° F. These conditions of becoming brittle when cold and fluid when hot must be dealt with in roofing manufacture utilizing bituminous or asphaltic materials. A certain amount of softening occurs in the roof in summer temperatures and the roofing becomes more brittle than is desirable under winter temperatures. This makes it necessary in laying roofing in cold weather in many cases

2

to be careful in handling the sheets or the shingles to prevent severe bending.

A quality which is desirable in such roofing is that for a given thickness of the sheet and weight of the sheet per unit of area, the sheet shall have a certain amount of stiffness without being so brittle that the saturated sheet or the saturated and coated sheet, for example when rolled in a roll, will crack when unrolled or bent slightly in erection. This compromise is secured in the manufacture of roofing with a felt base impregnated with saturants and coated with bituminous material by a compromise between rigidity which will prevent blowing-up in the wind of the sheet or shingles made therefrom and flexibility to prevent cracking of the sheet and its coating and to permit bending as above mentioned.

It has been proposed heretofore to treat a fibrous base sheet with asphalts or other bituminous materials having the characteristic of being very stiff at ordinary temperatures. Such products have been made in the form of flat sheets as backing sheets for roofing and covering materials. It also has been proposed to impregnate felted sheets in various forms with resinous materials such as shellac, rosin, natural and synthetic resins of various kinds, both thermoplastic and thermo setting. It further has been proposed to incorporate at the beaters in the paper-making process a thermoplastic resin so that this thermoplastic resin in divided form will be distributed throughout the felted structure of the dry felt as it leaves the paper machine preparatory to being impregnated with a bituminous saturant such as asphalt. The amount of such thermoplastic resin which may thus be incorporated in a felted structure is limited because of the method of its incorporation. Because ordinary methods in a paper-making process require suspension in a large amount of water such a resin could not be incorporated at the beater in an amount substantially in excess of 50% of the fiber weight in the felted sheet.

It is an object of the invention to produce a covering material which will have a substantial stiffness under a fairly wide range of temperatures, particularly the range of atmospheric temperatures experienced throughout the year.

It is also an object of the invention to secure in such a product a resistance to cracking or breaking under flexing stress.

It is a further object of the invention to accomplish these results in a sheet utilizing ordinary felt base materials.

It is a further object of the invention to secure

these properties in a rigid sheet material which will afford adequate resistance to the weather and to the action of light and heat.

According to the invention in its broad aspects a felted sheet, preferably as ordinarily made in the paper-making process, is impregnated with a thermoplastic resin to secure the desired stiffening of the felted sheet and resistance to softening under high temperatures. The sheet also may be impregnated with a bituminous material, particularly asphalt, which will afford weather resistance and at the same time provide a desirable resistance to cracking. A characteristic of such a bituminous material or such an asphalt for the purposes of the invention is that it shall have a low penetration, that is, the quality of maintaining its solidity and resistance to plastic flow or deformation at ordinary temperatures and below ordinary temperatures. Such a characteristic in an asphalt is secured, however, at the expense of increased thermal susceptibility. Thus at the higher temperatures to which such covering materials may be subjected such an asphalt would tend to become more plastic and of greater fluidity than is desirable. A sheet impregnated with such an asphalt would become too flexible and lose its resistance to bending. In some cases at the higher temperatures, such as may be experienced in tropical countries, the asphalt might ooze or run from the sheet. In view also of the purpose of the invention to provide a sheet material which will have structural characteristics, it is important that the rigidity of the sheet shall be substantially maintained throughout the range of temperatures to which the structure is subjected and that the fluid condition of the impregnating materials be not developed.

The function of the thermoplastic resin above referred to, therefore, is that it shall coact with the thermoplastic bituminous material, commonly asphalt, to maintain the rigidity of the sheet and prevent flow and softness at the higher temperatures to which the sheet is to be subjected. Resins of various kinds may be used, examples of which will be hereafter given, but a resin is chosen which substantially will maintain its penetration without great variation throughout the ordinary range of temperatures above given, viz.: 40° and 150° F. Particularly with the resinous material commercially known as Vinsol the penetration remains substantially constant throughout this range. Thus with a felted sheet impregnated with both the resin and the asphalt the cooperation of these two impregnating materials secures the qualities above described which are desirable for a structural sheet.

According to the invention the felted sheet is impregnated with the impregnating materials in molten condition. It is common practice to heat asphalt to fluid condition for impregnating felted sheets in roofing manufacture. It is further within the knowledge and skill of the art to impregnate felted sheets with resins in molten condition. In the practice of the invention these impregnating materials may be mixed together during the operation of melting them so that they may be delivered to or applied to the dry felt simultaneously as a mixture. Within the scope of the invention, however, these materials may be applied to the sheet separately, either one of them before the other, to impregnate the sheet with the desired or requisite amount of each of the impregnating materials.

By the method of impregnating a sheet with the resin and with the asphalt in molten condi-

tion a much higher percent of impregnation may be secured than by incorporating the materials at the beater, for example. Thus it is possible to impregnate an ordinary dry felt intended for roofing manufacture with molten asphalt in the amount of 175% to 200% or more of asphalt based on the weight of the dry felt. It is also possible to impregnate such a felt with the resin in the amount of 175% to 200% or more. For the purpose of the invention the amount of either impregnating material may be varied between 25% and 75% of the total amount of impregnating material. Thus the amount of either ingredient based on the weight of the dry felt, when for example the total impregnation is 200%, would be between 50% and 150%. These proportions and relations of the impregnating materials represent those which are preferable for securing the requisite cooperation of the two materials to obtain the two otherwise opposed characteristics in the sheet, viz.: rigidity and resistance to cracking. With a greater amount of the resin and therefore less of the asphalt, the sheet may become too brittle and too subject to cracking. With greater amounts of asphalt and less of resin insufficient stiffness for structural purposes of the sheet may result.

For the purposes of the invention the asphalts for impregnating the felted sheet may have ranges of penetration and melting point (softening point) as in the following table:

Table I

|                       | Available Range | Preferred Range |
|-----------------------|-----------------|-----------------|
| Penetration @ 77° F.  | 0-10            | 0-2             |
| Penetration @ 115° F. | 5-50            | 5-10            |
| Softening point, °F.  | 150-225         | 175-200         |

The penetration test as given in the above table is made by the American Society for Testing Materials Test D5—25, as given in the 1939 Standards, Part II, Non-Metallic Materials—Constructional, page 412, Method of Testing for Penetration of Bituminous Materials.

For practical reasons asphalts will be used for the purposes of the invention as in ordinary roofing manufacture which have a flash point not substantially less than 450° F. to prevent ignition causing fire. The asphalts may be selected as in roofing manufacture so that their viscosity at temperatures to which they may be heated above the melting point, namely 350°-450° F. without the risk of burning the base felt will secure the necessary fluidity for impregnating the felt and to secure the proper degree of saturation thereof in the ordinary processes and with the ordinary apparatus used in manufacture of roofing.

Also for the purpose of the invention these properties for the thermoplastic resin may lie within the following ranges:

Table II

|                       | Available Range | Preferred Range |
|-----------------------|-----------------|-----------------|
| Melting point, °F.    | 200-400         | -----           |
| Softening point, °F.  | 200-300         | -----           |
| Penetration @ 77° F.  | 0-4             | 0-2             |
| Penetration @ 150° F. | 0-25            | 0-7             |

The penetration for the resin known as Vinsol which will be hereafter further described and which is particularly suitable for the purposes of the invention was found to be substantially be-

tween 0 and 2 for all the temperatures at which tests were made, namely 77°, 115°, 135°, and 150° F. The melting point of this Vinsol resin is about 240° F. and the softening point 235° F.

The method of test of penetration for the resins is the same as that referred to above, namely the American Society for Testing Materials test for asphalt, except that in all cases the weight used to effect the penetration was 100 grams and the time 5 seconds for all temperatures. This modification of the test was adapted in view of the low penetration value of these resins.

The respective materials, i. e., asphalt and resin, selected to have these characteristics and used as impregnating materials in the roofing felt make it possible to secure in the finished sheet a product which will have the requisite stiffness at the ordinary high temperature which such roofing may acquire under summer sun, viz., of the degree of 175° F., and also not to become too brittle for handling and under load when placed in the structure at low winter temperatures.

A sheet of felt impregnated with the two kinds of materials, as above described, may be used for producing corrugated sheets. For this purpose the sheets may be impregnated with a mixture of molten resin and asphalt, and while the sheet is still hot may be pressed in a corrugated mold or other suitable mechanical device formed with the corrugations or with such other contour as will produce a mechanical form desired for the structural purpose. The corrugated sheet may then be allowed to cool to permit the thermoplastic content thereof to set. The result will be a corrugated sheet material which is of marked stiffness, not only because its corrugated form is maintained by the impregnating materials but also because of the inherent stiff character of the impregnated and set sheet itself. Such a corrugated sheet, moreover, will have weather-resisting properties by virtue of the asphalt impregnation and will be resistant to cracking or breaking because of the presence of the asphalt.

The sheet material of the invention produced in the manner above described, if desired, may be further treated with a weather and water resisting coating, such as asphalt, applied to the surface of the sheet. The impregnated sheet without asphalt coating thereon may have applied thereto a coating of metallic paint, such as aluminum paint, in order to afford heat reflection or the asphalt coated impregnated sheet may be coated with a metallic paint or may be surfaced with metallic flakes or powder. The asphalt coated sheet in some cases may be surfaced with mineral particles, such as those ordinarily applied to roofing sheets.

Ordinary roofing felts are particularly desirable for the purposes of the invention because they may be made in the paper-making process commonly used in roofing manufacture. For some purposes, however, such roofing felts which ordinarily vary in caliper from .025" to .080" will not as a single sheet provide sufficient thickness for the covering in the form of a flat sheet or as a corrugated sheet. Two or more of such roofing felts impregnated in accordance with the invention with a composite resin and asphalt material, therefore, may be laminated together to secure the increased thickness. Preferably these sheets are laminated together with an adhesive, especially asphalt, binding them together. Moreover it is the particular advantage of the lami-

nated form of the invention that the rigidity desired is obtained by virtue of the composite impregnating material but that the tendency to crack or to wrinkle at the surface of the sheet is reduced because of the limitation of the thickness of the laminations. This avoidance of cracking or wrinkling is thought to be due in part to the interposed layer of the plastic adhesive material between the laminations which layer, while holding the sheets strongly, reduces because of its plastic quality the amount of stretch or of compression at the surfaces of the individual laminations which produces cracking and wrinkling. This characteristic is especially desirable for the formation of corrugated sheets because in the process of forming the corrugations the amount of stretch which takes place in each of the laminations at each corrugation is thus limited. The impregnated sheet thus remains substantially in the form in which it was produced and the cooperation of the impregnating resin and the impregnating asphalt with each other and with the fibrous structure of the felt remains substantially undisturbed. There being no substantial cracking or wrinkling in the coated impregnated sheet, the weather-resisting property and the structural characteristic thereof thus are maintained.

The thermoplastic resins utilized in the invention of which Vinsol, above mentioned, is a commercial example, may be natural resins or synthetic resins which have the physical properties given in Table II above. As examples of such resins may be given the following:

Table III

|                      | Softening Point,<br>°F. | Melting<br>Point,<br>°F. |
|----------------------|-------------------------|--------------------------|
| East India Macassar  | 214-252                 | 261-313                  |
| East India Singapore | 228-252                 | 280-325                  |
| Batu East India      | 232-270                 | 320-356                  |
| Black East India     | 237-257                 | 318-327                  |
| Ester Gum            | Not less than 200       | 212-219                  |
| Pontianak            | 203-275                 | 259-336                  |

By ester gum is commonly understood an ester of rosin and glycerine, this product being well known in the varnish industry.

In addition to the above and preferred for the purposes of the invention the resin known as Vinsol which is commercially available has a low penetration as given in connection with Table II above and also has a low susceptibility. This resin may be melted, however, at about 240° F. and may be used in this melted condition to impregnate the felt in the same manner as is practiced with asphalt in roofing manufacture. The fluidity of the resin necessary for impregnation may be attained above the melting point but below the normal impregnating temperatures of between 350° and 450° F. as in the ordinary roofing manufacture. The resin in the melted condition is miscible with melted asphalt. If desired, however, the materials in sufficiently divided form may be mixed dry and then melted. The functions which have been referred to above for the two types of impregnating materials for the purposes of the invention may be secured by either method of preparation for impregnation.

Vinsol is prepared by extracting from the wood of stumps of southern long-leaf pine by the use of selective solvents the resinous materials contained in the wood. The stumps are first chipped and digested with benzene. The materials thus

dissolved in the processes of digestion are fractionated to remove the lighter fractions, that is, the solvent, turpentine, pine oil, etc. The residue remaining from the fractionation is a mixture of the Vinsol resin and other resins.

This composite material is then subjected to a further extraction process which consists of successive treatments with two immiscible solvents, furfural and naphtha. The Vinsol resin is very soluble in furfural whereas the other resins are not. Successive washings are made to purify the Vinsol resin which may be secured in the solid state by evaporation of the furfural solvent. The Vinsol resin may be defined as the extractive product derived by furfural extraction of the residue from the benzene extraction of chips from stumps of southern longleaf pine.

Thus the invention may provide a water-resistant covering material in different forms which, because of the composite impregnation, are of low thermal susceptibility at the same time having the requisite rigidity, resistance to fracture and strength for building purposes. Moreover, such sheets may be made penetrable for fasteners so as to be readily fastened to the supporting structure by the fasteners driven therethrough. The sheets thus may be used as are sheets of ordinary roofing materials or as are sheets of corrugated sheet metal. In the case of flat sheets of the invention the fasteners, if desired, may be sealed with a sealing cement, as in some cases is done with roofing sheets. In the case of the corrugated sheets the fasteners preferably are driven through the sheet at the peak of the corrugation so that the water will shed from the fastener. Moreover, as in applying corrugated sheet metal, nails having a flexible or deformable washer may be used. By virtue of the plastic characteristic of the roofing material itself, or the asphalt coating carried thereby, such fasteners may become slightly embedded in the surface of the sheet or the impregnating or the coating materials may close around the fastener by plastic flow to assist in securing water-tightness.

I claim:

1. Sheet material of low susceptibility to

change in flexibility throughout a temperature range of from low winter temperatures to about 175° F. adapted for use as roofing material comprising a base of felted fibrous material and impregnating material incorporated by absorption in said base and comprising pressure tar asphalt and a resin which is the portion of the resinous material of southern long-leaf pine which is soluble in benzene and in furfural but is insoluble in naphtha, each of said impregnating materials comprising from about 25% to about 75% by weight of the impregnating material.

10 2. Sheet material comprising a base of felted fibrous material, and impregnating material incorporated by absorption in said base and comprising a resin which is the portion of the resinous material of southern long-leaf pine which is soluble in benzene and in furfural but is insoluble in naphtha and pressure tar asphalt having a penetration value at 115° F. of between 5 and 50 and a softening point between 150° F. and 225° F., with each ingredient comprising from 25% to 75% by weight of the impregnating material.

25 MICHELE CROCE.

#### REFERENCES CITED

The following references are of record in the file of this patent:

#### UNITED STATES PATENTS

| Number       | Name         | Date          |
|--------------|--------------|---------------|
| 202,902      | Warren       | Apr. 23, 1878 |
| 1,849,867    | Eckert       | Mar. 15, 1932 |
| 35 1,949,255 | Keller       | Feb. 27, 1934 |
| 2,094,709    | Kinney       | Oct. 5, 1937  |
| 2,105,087    | Lutz         | Jan. 11, 1938 |
| 2,188,204    | Marc         | Jan. 23, 1940 |
| 2,188,478    | Lynn         | Jan. 30, 1940 |
| 40 2,204,772 | Rivkin       | June 18, 1940 |
| 2,223,289    | Lyons        | Nov. 26, 1940 |
| 2,346,947    | Schlaanstine | Apr. 18, 1944 |

#### OTHER REFERENCES

45 Vinsol Resin, Its Characteristics and Some Suggested Uses, p. 18, pub. 1937, Hercules Powder Co., Wilmington, Del.